

## UNITED STATES PATENT OFFICE

2,448,247

## TREATMENT OF TEXTILES WITH ACYLOXY-SUBSTITUTED AROMATIC ACID SALTS

Carl R. Bellwood, Ridgefield, N. J., assignor to The Cravette Company, U. S. A., Hoboken, N. J., a corporation of New Jersey

No Drawing. Application March 17, 1948,  
Serial No. 15,492

10 Claims. (Cl. 8—115.5)

1

This application is a continuation in part of my pending application Serial Number 496,613, filed July 29, 1943, now abandoned.

This invention relates to the treatment of cellulosic and proteinic fibers, and fabrics made from such fibers, to render them to an unusual degree persistently water repellent when repeatedly subjected to the customary normal washing and dry cleaning. Accordingly, garments made of such textiles (cotton, rayon, linen, jute, wool, silk, manipulated protein like casein fiber, synthetic polymers like nylon, etc., etc.), when treated by this process offer serviceable protection against wetting by rain or snow, even after being dry cleaned or washed many times. In addition, cloth treated according to this process is not substantially harmed as to "hand" or "drapery"; in fact, in many instances it is actually improved in those respects. There is the further advantage that, if desired in any particular case, the fibers processed as herein suggested, may be restored to substantially the condition they were in before the water-repellent quality was imparted to them. And finally, the ingredients used in the preparation of the materials employed in the process are normally readily available and comparatively cheap (some of them may be found on the market), and the technique of the application of the compounds to the cloth is simple and involves relatively little time, effort and expense.

I have discovered that certain substituted aliphatic esters, under proper conditions, will apparently undergo a reaction with the textile fibers, with the result that the water repellency of the fiber or any fabric made from this fiber is greatly increased; in addition, this water-repellent quality is maintained by the fiber or fabric even after many dry cleanings or washings of the type commonly employed in commercially cleaning such fabric or garment made therefrom.

Examples of starting materials that I may use in preparing the reaction compound are as follows:



Ortho stearoxybenzoic acid



Ortho lauryloxybenzoic acid



Para stearoxybenzoic acid



Para lauryloxybenzoic acid

2

Preparation of starting material  
and reaction compound

302 grams of stearyl chloride and 138 grams of ortho hydroxy benzoic acid or para hydroxy benzoic acid are heated together. During the heating process nitrogen which has been thoroughly dried of moisture is bubbled through the reaction mixture to liberate the hydrogen chloride. Heating is continued until evolution of hydrogen chloride ceases. The resulting compound, ortho stearoxybenzoic acid or para stearoxybenzoic acid, which may be called the starting material, is then cooled. 1 gram of this is dissolved in 99 cc. of water containing 0.2 gram of sodium hydroxide. The pH of the resulting solution is about 8-10. The finished reaction compound so prepared is presumably an approximately 1% solution of the sodium salt of ortho stearoxybenzoic acid or of the sodium salt of para stearoxybenzoic acid. In the same way solutions of the 35 alkali-metal salts of the homologues of ortho stearoxybenzoic acid or para stearoxybenzoic acid (for example, ortho or para lauryloxybenzoic acid—resulting from a variation in the length of the acyloxy radical—and 2-stearoxy-3-methylbenzoic acid—resulting from a variation of the aromatic nucleus) may be prepared. Also, in the 40 45 50 55

same way analogues of ortho stearyl oxybenzoic acid, para stearyl oxybenzoic acid, ortho lauryl oxybenzoic acid, and para lauryl oxybenzoic acid may be prepared among polynuclear compounds such as—

- 3-stearyl oxy-2-naphthoic acid;
- 2-stearyl oxy-3,6-naphthalenedisulfonic acid;
- 1-stearyl oxy-4-naphthalenesulfonic acid;
- 3-lauryl oxy-2-naphthoic acid;
- 2-lauryl oxy-3,6-naphthalenedisulfonic acid;
- 1-lauryl oxy-4-naphthalenesulfonic acid.

The behavior of these and their analogues and homologues is roughly equivalent.

The starting materials referred to are free acids. The reaction compound is made by bringing the free acid into solution by the addition of alkali. This process forms a solution of the alkali-metal salt of the free acid, said alkali-metal salt being herein referred to as the reaction compound.

By way of further example: 5 grams of the ortho stearyl oxybenzoic acid or of the para stearyl oxybenzoic acid may be dissolved in 95 cc. of water containing 1 gram of sodium hydroxide. The pH of the resulting solution is about 8 to 10, at any rate on the alkaline side to the extent that the compound is dissolved and so that application to the fabric is facilitated. The finished reaction compound so prepared is presumably an approximately 5% solution of the sodium salt of ortho stearyl oxybenzoic acid or of para stearyl oxybenzoic acid. Similarly, 5% solutions may also be prepared from homologues and analogues, which have already been discussed in connection with a 1% solution.

Pieces of cotton poplin and gabardine were dipped in the 1% solution and another set was dipped in the 5% solution, prepared as above. In each case the percentage absorption was about 80% after the samples were passed through squeeze rollers. Thus, in the case of the 1% solution the amount of active ingredient present in the cloth was 0.8% based on the dry weight of the cloth. In the case of the 5% solution, the amount of active ingredient present in the cloth was 4.0% based on the dry weight of the cloth. Each example was dried at 120° F. and baked at 300° F. The sample was then given a wash in water to remove products of the reaction.

Each sample was subjected to water-repellency tests as outlined in the American Association of Textile Chemists and Colorists Yearbook, vol. XIX (1942) pages 255/263, and was found to possess a high degree of water repellency with a spray test rating of 90. Each sample was subjected to several dry cleaning treatments employing a machine as outlined in Federal Specification CCC-T-191a, section XIII, paragraph 4, and following the procedure outlined in Federal Specification P. Q. D. No. 1, section F, paragraph 3d, and was found to retain most of its water repellency according to the above testing methods. Each sample was subjected to several laundering treatments as outlined in the American Association of Textile Chemists and Colorists Yearbook, vol. XIX (1942), pages 244 and 245, and was found to retain most of its original water repellency.

The drying may be carried on at about 120° F., and the baking at a temperature of about 275–300° F. for about 5–15 minutes. The drying and baking may be carried out as parts of a continuous operation in a single piece of apparatus, or they may be carried out separately in separate apparatus. The fabric may be subjected to ap-

proximately the same conditions, and satisfactory results obtained, by passing the wet web of fabric into a dry chamber in which the air is circulated and is maintained at preferably from 300°–310° F., the web being continuously moved through the chamber at a speed which will cause any given portion of the fabric to remain in the chamber for approximately 15 minutes. For about the first 5 minutes of such treatment the fabric dries, and for the remainder of the time it bakes. However the drying be done, I prefer that the fabric, after having the moisture removed therefrom, be subjected to a baking temperature of at least 275° F. and preferably 300° F.

Examples have been given in which the immersion of the cloth was in a solution of the sodium salt of ortho stearyl oxybenzoic acid or of para stearyl oxybenzoic acid adjusted to a pH of about 8–10. I prefer a solution of the order of 5%. Instead of using the sodium salt, I may use the salt of potassium or other alkali metal. Also, I might use ortho or para benzenesulfonic acid derivatives, or naphthalenesulfonic acid derivatives, or naphthoic acid derivatives, or compounds having acyloxy aliphatic groups containing 8–20 carbon atoms, in place of the ortho or para stearyl oxybenzoic acid specified in the example. With reference to the maximum number of carbon atoms in the acyloxy aliphatic group, I have never reached an upper limit. As the number of carbon atoms is increased, it could be expected that a point would be reached where the compound would become relatively inactive. However, I have successfully used compounds having as many as 26 carbon atoms in the acyloxy aliphatic group, e.g. ortho cetyl oxybenzoic acid.

Broadly, a reaction compound as herein contemplated may be said to answer to the formula



where

- 40 (a) Ar is a divalent aromatic nucleus such as  $\text{C}_6\text{H}_4$ ; or  $\text{C}_{10}\text{H}_8$ ; or their homologues
- (b) R is a saturated aliphatic chain containing 7 or more carbon atoms
- (c) X is an acid group such as  $(-\text{COO})^-$  or  $(-\text{SO}_2\text{O})^-$
- (d) Me is an alkali-metal ion such as sodium or potassium.
- (e) And groups (1) and (2) are in ortho or para relationship in the benzene compound, and in two-three or one-four relationship in the naphthalene series—

the other symbols having their usual technical meanings.

60 Or, the reaction compound may be said to comprise, generally, a soluble alkali-metal salt of an acyloxy-substituted aromatic acid, where the acyloxy group is aliphatic and may contain more than 7 carbon atoms, adjusted to a pH of the order of about 8–10.

While I have spoken of the textile fabrics and fibers in general terms, it is to be understood that I contemplate the treatment of dyed, as well as undyed material, provided, of course, that there is nothing in the dye that inhibits or substantially modifies the action of, or is otherwise incompatible with the chosen reaction compound.

It is within the contemplated application of my invention to combine two or more of the reaction compounds herein mentioned, for the pro-

duction of a multiple or superreaction compound, where trial shows that such combinations produce repellency or incidental beneficial effects greater than those resulting from the use of individual constituent reaction compounds.

I claim:

1. The method of treating fibers and fabrics of the kind set forth to render them water repellent, which consists in subjecting them to the action of an aqueous solution of a compound answering to the formula



where

- (a) Ar is a divalent aromatic nucleus selected from the group consisting of  $C_6H_4$  and  $C_{10}H_8$
  - (b) R is a saturated aliphatic chain containing 7 or more carbon atoms
  - (c) X is selected from the group consisting of  $(-COO^-)$  and  $(-SO_2O^-)$
  - (d) Me is an alkali metal
  - (e) And groups (1) and (2) are in ortho or para relationship in the benzene compound and in two-three or one-four relationship in the naphthalene series—

the other symbols having their usual technical meaning; and then drying and baking the material being treated.

2. The method of treating fibers and fabrics of the kind set forth to render them water repellent, which consists in subjecting them to the action of an aqueous solution of a compound answering to the formula



where

- (a) Ar is the divalent aromatic nucleus  $C_6H_4$
  - (b) R is a saturated aliphatic chain containing 7 or more carbon atoms
  - (c) X is selected from the group consisting of  $(-COO^-)$  and  $(-SO_2O^-)$
  - (d) Me is an alkali metal
  - (e) And groups (1) and (2) are in ortho or para relationship—

the other symbols having their usual technical meaning; and then drying and baking the material being treated.

3. The method as in claim 2 in which the material is dried at approximately 120° F. and baked at about 275°-300° F.

4. The method as in claim 2 in which the material is dried at 120° F. and baked at 300° F.

5. The method of treating fibers and fabrics of the kind set forth to render them water repellent, which consists in subjecting them to the action of an aqueous solution of a compound answering to the formula



where

- (a) Ar is the divalent aromatic nucleus  $C_{10}H_8$   
 (b) R is a saturated aliphatic chain containing 7 or more carbon atoms  
 15 (c) X is selected from the group consisting of  $(-COO^-)$  and  $(-SO_2O^-)$   
 (d) Me is an alkali metal  
 (e) And groups (1) and (2) are in two three

(c) And groups (1) and (2) are in two-three or one-four relationship—

20 the other symbols having their usual technical meaning; and then drying and baking the material being treated.

6. The method as in claim 5 in which the material is dried at approximately 120° F. and baked at about 275°-300° F.

7. The method as in claim 5 in which the material is dried at 120° F. and baked at 300° F.

30 8. The method of treating fibers and fabrics of the kind set forth to render them water repellent, which consists in subjecting them to the action of an aqueous solution of an alkali-metal salt of ortho stearyl oxybenzoic acid, and then drying and baking the material being treated.

35 9. The method of treating fibers and fabrics of the kind set forth to render them water repellent, which consists in subjecting them to the action of an aqueous solution of an alkali-metal salt of 3-stearyloxy-2-naphthoic acid, and then drying and baking the material being treated.

10 10. The method of treating fibers and fabrics  
of the kind set forth to render them water repellent, which consists in subjecting them to the action of an aqueous solution of an alkali-metal salt  
45 of 1-stearyloxy-4-naphthalenesulfonic acid, and then drying and baking the material being treated.

CARL R. BELLWOOD.

#### REFERENCES CITED

The following references are of record in the file of this patent:

UNITED STATES PATENTS

| 55 | Number    | Name                   | Date          |
|----|-----------|------------------------|---------------|
|    | 1,916,776 | Steindorff et al. .... | July 4, 1933  |
|    | 2,125,072 | Kern .....             | July 26, 1938 |
|    | 2,146,308 | Shipp .....            | Feb. 7, 1939  |
|    | 2,146,392 | Shipp .....            | Feb. 7, 1939  |
| 60 | 2,313,741 | Engelmann et al. ....  | Mar. 16, 1943 |
|    | 2,337,924 | Platz et al. ....      | Dec. 28, 1943 |